



US007678856B2

(12) **United States Patent**  
**Goulet et al.**

(10) **Patent No.:** **US 7,678,856 B2**  
(b5) **Date of Patent:** **Mar. 16, 2010**

(54) **BINDERS CURABLE AT ROOM TEMPERATURE WITH LOW BLOCKING**

(75) Inventors: **Mike Thomas Goulet**, Neenah, WI (US); **Tracy Ho Mathews**, Neenah, WI (US); **Stacey Lynn Pomeroy**, DePere, WI (US); **Maurizio Tirimacco**, Appleton, WI (US)

(73) Assignee: **Kimberly-Clark Worldwide Inc.**, Neenah, WI (US)

(\*) Notice: Subject to any disclaimer, the term of this patent is extended or adjusted under 35 U.S.C. 154(b) by 163 days.

(21) Appl. No.: **11/901,427**

(22) Filed: **Sep. 17, 2007**

(65) **Prior Publication Data**

US 2008/0006381 A1 Jan. 10, 2008

**Related U.S. Application Data**

(62) Division of application No. 10/893,094, filed on Jul. 15, 2004, now Pat. No. 7,297,231.

(51) **Int. Cl.**

**C08F 220/02** (2006.01)

(52) **U.S. Cl.** ..... **524/500**; 524/502; 524/519; 524/521; 524/522; 524/539

(58) **Field of Classification Search** ..... **524/500, 524/502, 519, 521, 522, 527, 539**

See application file for complete search history.

(56) **References Cited**

U.S. PATENT DOCUMENTS

|             |         |                 |
|-------------|---------|-----------------|
| 2,624,245 A | 1/1953  | Cluett          |
| 3,011,545 A | 12/1961 | Welsh et al.    |
| 3,017,317 A | 1/1962  | Voigtman et al. |
| 3,096,228 A | 7/1963  | Day et al.      |
| 3,260,778 A | 7/1966  | Walton          |
| 3,301,746 A | 1/1967  | Sanford et al.  |

|             |         |                 |
|-------------|---------|-----------------|
| 3,329,556 A | 7/1967  | McFalls et al.  |
| 3,338,858 A | 8/1967  | Strasser et al. |
| 3,359,166 A | 12/1967 | Freuler et al.  |
| 3,416,192 A | 12/1968 | Packard         |
| 3,426,405 A | 2/1969  | Walton          |
| 3,554,863 A | 1/1971  | Hervey et al.   |
| 3,630,837 A | 12/1971 | Freuler         |
| 3,660,338 A | 5/1972  | Economou        |
| 3,686,151 A | 8/1972  | Keim            |
| 3,700,623 A | 10/1972 | Keim            |
| 3,772,076 A | 11/1973 | Keim            |
| 3,821,068 A | 6/1974  | Shaw            |
| 3,833,531 A | 9/1974  | Keim            |

(Continued)

FOREIGN PATENT DOCUMENTS

DE 34 41 883 A1 5/1986

(Continued)

OTHER PUBLICATIONS

Chan, "Wet Strength Resins and Their Application" TAPPI Press, 1994, Chapter 2, pp. 13-22.\*

(Continued)

*Primary Examiner*—Eric Hug

*Assistant Examiner*—Dennis Cordray

(74) *Attorney, Agent, or Firm*—Gregory E. Croft

(57) **ABSTRACT**

Topically-applied binder materials for imparting wet strength to soft, absorbent paper sheets, such as are useful as household paper towels and the like, include an azetidinium-reactive polymer, such as a carboxyl-functional polymer, an azetidinium-functional polymer and, optionally, a component useful for reducing sheet-to-sheet adhesion (blocking) in the product. These binder materials can be cured at ambient temperature over a period of days and do not impart objectionable odor to final product when wetted.

**18 Claims, 1 Drawing Sheet**



# US 7,678,856 B2

Page 2

## U.S. PATENT DOCUMENTS

|               |         |                             |                |          |                         |
|---------------|---------|-----------------------------|----------------|----------|-------------------------|
| 3,844,880 A   | 10/1974 | Meisel, Jr. et al.          | 5,709,775 A    | 1/1998   | Trokan et al.           |
| 3,879,257 A   | 4/1975  | Gentile et al.              | 5,716,603 A    | * 2/1998 | Chen et al. .... 424/61 |
| 3,903,342 A   | 9/1975  | Roberts, Jr.                | 5,776,312 A    | 7/1998   | Trokan et al.           |
| 3,926,716 A   | 12/1975 | Bates                       | 5,804,036 A    | 9/1998   | Phan et al.             |
| 3,949,014 A * | 4/1976  | Maki et al. .... 525/187    | 5,820,730 A    | 10/1998  | Phan et al.             |
| 3,994,771 A   | 11/1976 | Morgan, Jr. et al.          | 5,830,321 A    | 11/1998  | Lindsay et al.          |
| 4,000,237 A   | 12/1976 | Roberts, Jr.                | 5,837,103 A    | 11/1998  | Trokan et al.           |
| 4,072,557 A   | 2/1978  | Schiel                      | 5,840,403 A    | 11/1998  | Trokan et al.           |
| 4,090,385 A   | 5/1978  | Packard                     | 5,843,279 A    | 12/1998  | Phan et al.             |
| 4,125,659 A   | 11/1978 | Klowak et al.               | 5,846,379 A    | 12/1998  | Ampulski et al.         |
| 4,132,695 A   | 1/1979  | Burkholder                  | 5,855,739 A    | 1/1999   | Ampulski et al.         |
| 4,144,122 A   | 3/1979  | Emanuelsson et al.          | 5,871,887 A    | 2/1999   | Trokan et al.           |
| 4,152,507 A   | 5/1979  | Yamamoto                    | 5,872,181 A    | 2/1999   | Daniels et al.          |
| 4,158,594 A   | 6/1979  | Becker et al.               | 5,877,239 A    | 3/1999   | Craun et al.            |
| 4,208,459 A   | 6/1980  | Becker et al.               | 5,885,418 A    | 3/1999   | Anderson et al.         |
| 4,326,000 A   | 4/1982  | Roberts, Jr.                | 5,893,965 A    | 4/1999   | Trokan et al.           |
| 4,351,699 A   | 9/1982  | Osborn, III                 | 5,897,745 A    | 4/1999   | Ampulski et al.         |
| 4,440,597 A   | 4/1984  | Wells et al.                | 5,904,811 A    | 5/1999   | Ampulski et al.         |
| 4,442,833 A   | 4/1984  | Dahlen et al.               | 5,906,710 A    | 5/1999   | Trokan                  |
| 4,483,332 A   | 11/1984 | Rind                        | 5,908,889 A    | 6/1999   | Bailey et al.           |
| 4,507,173 A   | 3/1985  | Klowak et al.               | 5,919,556 A    | 7/1999   | Barnholtz               |
| 4,528,239 A   | 7/1985  | Trokan                      | 5,935,381 A    | 8/1999   | Trokan et al.           |
| 4,529,480 A   | 7/1985  | Trokan                      | 5,948,210 A    | 9/1999   | Huston                  |
| 4,529,489 A   | 7/1985  | McDonald et al.             | 5,989,682 A    | 11/1999  | Anderson                |
| 4,610,743 A   | 9/1986  | Salmeen et al.              | 5,990,377 A    | 11/1999  | Chen et al.             |
| 4,637,859 A   | 1/1987  | Trokan                      | 6,017,417 A    | 1/2000   | Wendt et al.            |
| 4,710,374 A   | 12/1987 | Grollier et al.             | 6,039,839 A    | 3/2000   | Trokan et al.           |
| 4,785,030 A   | 11/1988 | Noda et al.                 | 6,054,020 A    | 4/2000   | Goulet et al.           |
| 4,822,453 A   | 4/1989  | Dean et al.                 | 6,059,928 A    | 5/2000   | Van Luu et al.          |
| 4,859,527 A   | 8/1989  | Distefano                   | 6,063,449 A    | 5/2000   | Koskinen et al.         |
| 4,891,249 A   | 1/1990  | McIntyre                    | 6,083,346 A    | 7/2000   | Hermans et al.          |
| 4,919,877 A   | 4/1990  | Parsons et al.              | 6,096,152 A    | 8/2000   | Anderson et al.         |
| 4,944,960 A   | 7/1990  | Sundholm et al.             | 6,096,169 A    | 8/2000   | Hermans et al.          |
| 4,949,668 A   | 8/1990  | Heindel et al.              | 6,103,062 A    | 8/2000   | Ampulski et al.         |
| 4,996,091 A   | 2/1991  | McIntyre                    | 6,103,861 A    | 8/2000   | Staib et al.            |
| 5,124,188 A   | 6/1992  | Roe et al.                  | 6,117,270 A    | 9/2000   | Trokan                  |
| 5,129,988 A   | 7/1992  | Farrington, Jr.             | 6,117,492 A    | 9/2000   | Goldstein et al.        |
| 5,143,776 A   | 9/1992  | Givens                      | 6,120,642 A    | 9/2000   | Lindsay et al.          |
| 5,175,197 A * | 12/1992 | Gestner et al. .... 523/218 | 6,126,784 A    | 10/2000  | Ficke et al.            |
| 5,196,470 A   | 3/1993  | Anderson et al.             | 6,129,815 A    | 10/2000  | Larson et al.           |
| 5,200,036 A   | 4/1993  | Noda                        | 6,136,146 A    | 10/2000  | Phan et al.             |
| 5,213,588 A * | 5/1993  | Wong et al. .... 51/293     | 6,140,419 A    | 10/2000  | Barglik-Chory et al.    |
| 5,225,460 A   | 7/1993  | Sampath et al.              | 6,143,135 A    | 11/2000  | Hada et al.             |
| 5,264,468 A   | 11/1993 | Miyahara                    | 6,179,961 B1   | 1/2001   | Ficke et al.            |
| 5,312,863 A   | 5/1994  | Van Rheenen et al.          | 6,187,137 B1   | 2/2001   | Druecke et al.          |
| 5,324,561 A   | 6/1994  | Rezai et al.                | 6,187,139 B1   | 2/2001   | Edwards et al.          |
| 5,334,289 A   | 8/1994  | Trokan et al.               | 6,187,140 B1   | 2/2001   | Anderson et al.         |
| 5,342,875 A   | 8/1994  | Noda                        | 6,193,847 B1   | 2/2001   | Trokan                  |
| 5,366,785 A   | 11/1994 | Sawdai                      | 6,197,154 B1   | 3/2001   | Chen et al.             |
| 5,399,412 A   | 3/1995  | Sudall et al.               | 6,197,880 B1 * | 3/2001   | Nigam .... 524/845      |
| 5,429,686 A   | 7/1995  | Chiu et al.                 | 6,200,418 B1   | 3/2001   | Oriaran et al.          |
| 5,443,691 A   | 8/1995  | Phan et al.                 | 6,228,216 B1   | 5/2001   | Lindsay et al.          |
| 5,484,825 A   | 1/1996  | Dick et al.                 | 6,303,672 B1   | 10/2001  | Papalos et al.          |
| 5,494,554 A   | 2/1996  | Edwards et al.              | 6,309,527 B1   | 10/2001  | Broekhuis et al.        |
| 5,525,664 A * | 6/1996  | Miller et al. .... 524/845  | 6,319,312 B1   | 11/2001  | Luongo                  |
| 5,529,664 A   | 6/1996  | Trokan et al.               | 6,387,989 B1   | 5/2002   | Sulzbach et al.         |
| 5,529,665 A   | 6/1996  | Kaun                        | 6,395,957 B1   | 5/2002   | Chen et al.             |
| 5,547,710 A   | 8/1996  | Satgurunathan et al.        | 6,410,617 B1   | 6/2002   | Sulzbach et al.         |
| 5,556,509 A   | 9/1996  | Trokan et al.               | 6,420,013 B1   | 7/2002   | Vinson et al.           |
| 5,575,891 A   | 11/1996 | Trokan et al.               | 6,423,180 B1   | 7/2002   | Behnke et al.           |
| 5,593,545 A   | 1/1997  | Rugowski et al.             | 6,426,121 B1   | 7/2002   | Goldstein et al.        |
| 5,607,551 A   | 3/1997  | Farrington, Jr. et al.      | 6,462,159 B1   | 10/2002  | Hamada et al.           |
| 5,610,215 A   | 3/1997  | Nonweiler et al.            | 6,464,831 B1   | 10/2002  | Trokan et al.           |
| 5,614,061 A   | 3/1997  | Van Phan et al.             | 6,465,556 B1   | 10/2002  | Pratt et al.            |
| 5,614,597 A   | 3/1997  | Bower                       | 6,500,289 B2   | 12/2002  | Merker et al.           |
| 5,637,194 A   | 6/1997  | Ampulski et al.             | 6,506,696 B2   | 1/2003   | Goldstein et al.        |
| 5,656,132 A   | 8/1997  | Farrington, Jr. et al.      | 6,506,821 B1   | 1/2003   | Huver et al.            |
| 5,667,636 A   | 9/1997  | Engel et al.                | 6,533,978 B1   | 3/2003   | Wisneski et al.         |
| 5,672,248 A   | 9/1997  | Wendt et al.                | 6,534,151 B2   | 3/2003   | Merker                  |
| 5,674,590 A   | 10/1997 | Anderson et al.             | 6,534,177 B2   | 3/2003   | Kohlhammer et al.       |
| 5,679,222 A   | 10/1997 | Rasch et al.                | 6,576,091 B1   | 6/2003   | Cabell et al.           |
|               |         |                             | 6,586,520 B1   | 7/2003   | Canorro et al.          |

|              |     |         |                    |
|--------------|-----|---------|--------------------|
| 6,607,630    | B2  | 8/2003  | Bartman et al.     |
| 6,608,237    | B1  | 8/2003  | Li et al.          |
| 6,610,173    | B1  | 8/2003  | Lindsay et al.     |
| 6,660,362    | B1  | 12/2003 | Lindsay et al.     |
| 6,727,004    | B2  | 4/2004  | Goulet et al.      |
| 6,846,383    | B2  | 1/2005  | Tirimacco          |
| 6,918,993    | B2  | 7/2005  | Tirimacco          |
| 6,936,316    | B2  | 8/2005  | Nigam et al.       |
| 7,045,026    | B2  | 5/2006  | Lorenz et al.      |
| 2001/0005529 | A1  | 6/2001  | Owens et al.       |
| 2001/0024644 | A1  | 9/2001  | Kohlhammer et al.  |
| 2002/0107495 | A1  | 8/2002  | Chen et al.        |
| 2002/0117280 | A1  | 8/2002  | Howle et al.       |
| 2003/0059636 | A1* | 3/2003  | Nigam .....        |
| 2003/0079847 | A1  | 5/2003  | Howle et al.       |
| 2003/0112311 | A1* | 6/2003  | Naik et al. ....   |
| 2003/0121627 | A1* | 7/2003  | Hu et al. ....     |
| 2003/0199629 | A1* | 10/2003 | Gelman et al. .... |
| 2004/0007339 | A1  | 1/2004  | Tirimacco          |
| 2004/0018369 | A1  | 1/2004  | Goulet et al.      |
| 2004/0031578 | A1  | 2/2004  | Tirimacco          |
| 2004/0086726 | A1  | 5/2004  | Moline et al.      |
| 2004/0099388 | A1  | 5/2004  | Chen et al.        |
| 2004/0114012 | A1* | 6/2004  | Chu et al. ....    |
| 2004/0118531 | A1  | 6/2004  | Shannon et al.     |
| 2004/0118532 | A1  | 6/2004  | Sarbo et al.       |
| 2004/0118544 | A1  | 6/2004  | Tirimacco et al.   |
| 2004/0123963 | A1  | 7/2004  | Chen et al.        |
| 2004/0192136 | A1  | 9/2004  | Gusky et al.       |
| 2005/0004309 | A1  | 1/2005  | Gerst et al.       |
| 2005/0045292 | A1  | 3/2005  | Lindsay et al.     |
| 2005/0045293 | A1  | 3/2005  | Hermans et al.     |
| 2005/0045294 | A1  | 3/2005  | Goulet et al.      |
| 2005/0045295 | A1  | 3/2005  | Goulet et al.      |
| 2005/0247417 | A1  | 11/2005 | Tirimacco          |
| 2006/0014884 | A1  | 1/2006  | Goulet et al.      |
| 2006/0124261 | A1  | 6/2006  | Lindsay et al.     |
| 2007/0010153 | A1  | 1/2007  | Shaffer et al.     |
| 2007/0051484 | A1  | 3/2007  | Hermans et al.     |
| 2007/0102127 | A1  | 5/2007  | Hermans et al.     |
| 2007/0187056 | A1  | 8/2007  | Goulet et al.      |
| 2007/0194274 | A1  | 8/2007  | Goulet et al.      |
| 2008/0035288 | A1  | 2/2008  | Mullally et al.    |

## FOREIGN PATENT DOCUMENTS

|    |             |    |         |
|----|-------------|----|---------|
| DE | 43 05 727   | A1 | 9/1994  |
| EP | 0 135 231   | A1 | 3/1985  |
| EP | 0 140 404   | A1 | 5/1985  |
| EP | 0 618 005   | A2 | 10/1994 |
| EP | 0 662 542   | A1 | 7/1995  |
| EP | 0 549 925   | B1 | 8/1995  |
| EP | 0 694 578   | A2 | 1/1996  |
| EP | 0 661 030   | B1 | 7/2000  |
| EP | 1 180 559   | A1 | 2/2002  |
| EP | 1 082 391   | B1 | 6/2002  |
| EP | 1 316 432   | A1 | 6/2003  |
| GB | 2 006 296   | A  | 5/1979  |
| GB | 2 303 647   | A  | 2/1997  |
| WO | WO 92/16681 | A1 | 10/1992 |
| WO | WO 93/10732 | A1 | 6/1993  |
| WO | WO 97/44528 | A1 | 11/1997 |
| WO | WO 97/47227 | A1 | 12/1997 |
| WO | WO 98/37274 | A1 | 8/1998  |
| WO | WO 98/55695 | A1 | 12/1998 |
| WO | WO 99/10597 | A1 | 3/1999  |
| WO | WO 99/34057 | A1 | 7/1999  |
| WO | WO 99/34060 | A1 | 7/1999  |
| WO | WO 00/08077 | A1 | 2/2000  |
| WO | WO 00/66835 | A1 | 11/2000 |
| WO | WO 01/02644 | A1 | 1/2001  |
| WO | WO 01/14641 | A1 | 3/2001  |
| WO | WO 02/29154 | A2 | 4/2002  |

|    |                |    |         |
|----|----------------|----|---------|
| WO | WO 02/41815    | A2 | 5/2002  |
| WO | WO 02/100032   | A1 | 12/2002 |
| WO | WO 2004/005039 | A1 | 1/2004  |
| WO | WO 2004/009905 | A1 | 1/2004  |
| WO | WO 2004/037935 | A1 | 5/2004  |
| WO | WO 2005/021868 | A1 | 3/2005  |

## OTHER PUBLICATIONS

American Society for Testing Materials (ASTM) Designation: D1544-98, "Standard Test Method for Color of Transparent Liquids (Gardner Color Scale)," pp. 1-2, published Sep. 1998.

American Society for Testing Materials (ASTM) Designation: D5170-98, "Standard Test Method for Peel Strength ("T" Method) of Hook and Loop Touch Fasteners," pp. 702-704, published Mar. 1999. TAPPI Official Test Method T 402 om-93, "Standard Conditioning and Testing Atmospheres for Paper, Board, Pulp Handsheets, and Related Products," published by the TAPPI Press, Atlanta, Georgia, revised 1993, pp. 1-3.

TAPPI Official Test Method T 411 om-89, "Thickness (Caliper) of Paper, Paperboard, and Combined Board," published by the TAPPI Press, Atlanta, Georgia, revised 1989, pp. 1-3.

"Airflex 426 Emulsion," Air Products Polymers, L.P., 2-page brochure and Internet web page "[http://airproducts.com/polymers/controlled/product\\_description.asp?intRegionalMarketSegment=55...](http://airproducts.com/polymers/controlled/product_description.asp?intRegionalMarketSegment=55...)" printed Jul. 1, 2003, 2 pages and 1 page Specifications.

"Glycidyl Ethers," KEMI, National Chemicals Inspectorate, Sweden, Internet web page "[http://www.kemi.se/kemamne\\_eng/glycidetrar\\_eng.htm](http://www.kemi.se/kemamne_eng/glycidetrar_eng.htm)", viewed and printed Jul. 29, 2003, pp. 1-2.

Bhangale, Sunil M., "Epoxy Resins," Internet web page "<http://sunilbhangale.tripod.com/epoxy.html>", viewed and printed Jul. 29, 2003, pp. 1-4.

Blank, Werner J. et al., "Catalysis of the Epoxy-Carboxyl Reaction," *International Waterborne, High-Solids and Powder Coatings Symposium*, New Orleans, LA, Feb. 21-23, 2001, sponsored by the University of Southern Mississippi, Paper23\_ict1.doc, printed Aug. 8, 2001, 18 pages.

Carey, Francise A., "Reactions of Epoxides," *Organic Chemistry 4e Carey Online Learning Center*, Chapter 16: Ethers, Epoxides and Sulfides, McGraw Hill, 2000, Internet web page, "<http://www mhhe.com/physsci/chemistry/carey/student/olc/ch16reactionsepoxides.html>", viewed and printed Jul. 29, 2003, pp. 1-4.

Day, Dr. Richard, "Epoxy Resins," Internet web page, "<http://www2.umist.ac.uk/material/teaching/year2/ml260/epoxy.doc>", Feb. 26, 1998, viewed and printed Jul. 29, 2003, 10 pages.

DeVry, William E., "Latex Bonding Chemistry and Processes," *Nonwovens An Advanced Tutorial*, edited by Albin F. Turbak and Tyrone L. Vigo, TAPPI Press, Atlanta, GA, 1989, Chapter 5, pp. 51-69.

Donnelly, R.H. and Martti Kangas, "Dryad Technology—Implementing Spraying Technology in Paper and Board Manufacturing," *Paperi ja Puu—Paper and Timber*, vol. 83. No. 7, 2001, pp. 530-531.

Espy, Herbert H., "Alkaline-Curing Polymeric Amine-Epichlorohydrin Resins," *Wet-Strength Resins and Their Application*, edited by Lock L. Chan, Chapter 2, TAPPI Press, Atlanta, GA, 1994, pp. 14-44.

Moyer, W.W. Jr. and R.A. Stagg, "Miscellaneous Wet-Strength Agents," *Wet Strength in Paper and Paperboard*, TAPPI Monograph Series No. 29, Technical Association of the Pulp and Paper Industry, Mack Printing Company, Easton, PA, Chapter 8, 1965, pp. 105-125. Oinonen, Hannu, "Metso Introduces New Coating Method: Spray for Light-Weight Coating," *Parperi ja Puu—Paper and Timber*, vol. 83, No. 7, 2001, pp. 526-528.

Sabia, A.J. and R.B. Metzler, "The Role of Silicones in Woven and Nonwoven Fabric Applications," *Advances in Nonwoven Technology—Tenth Technical Symposium*, Inda, Association of the Nonwoven Fabrics Industry, New York, Nov. 17-19, 1982, pp. 284-293.

Zhao, Yaqiu and Marek W. Urban, "Novel STY/nBA/GMA and STY/nBA/MAA Core—Shell Latex Blends: Film Formation, Particle

Morphology, and Cross-Linking. 20. A Spectroscopic Study," *Macromolecules*, vol. 33, No. 22, 2000, pp. 8426-8434.

Smook, Gary A., Editor, "Manufacturing Techniques for Specific Paper and Board Grades," *Handbook for Pulp & Paper Technologists*, Second Edition, Angus Wilde Publications, Bellingham, WA, 1992, pp. 318-319.

\* cited by examiner



FIG. 1

## 1

## BINDERS CURABLE AT ROOM TEMPERATURE WITH LOW BLOCKING

This application is a divisional of U.S. Ser. No. 10/893,094 filed Jul. 15, 2004, now U.S. Pat. No. 7,297,231. The entirety of U.S. Ser. No. 10/893,094 is hereby incorporated by reference.

## BACKGROUND OF THE INVENTION

In the manufacture of certain bonded non-woven products, the use of topical binders to impart added strength to the final product is well known. An example of such a process is disclosed in U.S. Pat. No. 3,879,257 entitled "Absorbent Unitary Laminate-Like Fibrous Webs and Method for Producing Them" and issued Apr. 22, 1975 to Gentile et al., herein incorporated by reference. A problem associated with commercially available topical binders is that they require a highly elevated curing temperature to impart the desired strength, which in turn requires a curing oven or equivalent apparatus. These requirements add to the capital and manufacturing costs associated with the product. Also, some commercially available binders can emit hazardous air pollutants, such as formaldehyde, and the resulting product can exhibit an undesirable odor, particularly when wetted.

An improved binder system is disclosed in co-pending U.S. patent application Ser. No. 10/654,556 entitled "Low Odor Binders Curable at Room Temperature" filed Sep. 2, 2003 by Goulet et al. This binder system utilizes a mixture of an epoxy-reactive polymer and an epoxy-functional polymer. However, there remains a need to continually improve upon binder systems useful for the commercial production of paper towels, for example.

## SUMMARY OF THE INVENTION

It now has been discovered that binder systems involving the reaction between an azetidinium-reactive polymer and an azetidinium-functional cross-linking polymer, when topically applied to a fibrous web such as a paper web, particularly a tissue or paper towel basesheet, can cure at ambient or low temperature without emitting formaldehyde and without imparting objectionable odors to the resulting product. Furthermore, such binder systems exhibit additional commercial advantages, such as viscosity stability, ease of use and low cost. Specifically, these binder systems retain a low viscosity value for a prolonged period of time (weeks) compared to other low temperature cure binder systems which significantly increase in viscosity after several hours, which makes application of the binder more difficult. Regarding ease of use, the azetidinium-functional cross-linking polymer does not require an activation step using a strong base as is needed with some other binder systems, which makes it easier to prepare, safer to handle and reduces overall binder cost. Further in regard to cost, azetidinium-functional cross-linking polymers can be considerably less expensive than epoxy-functional resins due to the existing large commercial market for azetidinium-functional cross-linking polymers as wet end additives for paper.

Without being bound by theory, it is hypothesized that during and after drying of the paper web, the functional moiety on the latex polymer reacts with the azetidinium-functional reactant to form a covalently bonded polymer network. Simultaneously, it is also hypothesized that the azetidinium-functional reactant can also react with carboxylic acid or other functional groups present on the fiber surface to provide additional strengthening of the basesheet. In addi-

## 2

tion, for poly(aminoamide)-epichlorohydrin resins, the azetidinium functional group can self-crosslink with amine functional groups present on the resin. In addition, and also simultaneously, for binder formulations that contain cross-linking additives designed to reduce blocking, these cross-linking additives are activated during the thermal drying step and can react both with the latex polymer and/or the non-woven basesheet fibers to hold the polymer in place and reduce its ability to flow and increase blocking resistance characteristics of the bonded basesheet.

Hence, in one aspect the invention resides in an aqueous binder composition comprising an unreacted mixture of an azetidinium-reactive polymer and an azetidinium-functional cross-linking polymer, wherein the amount of the azetidinium-functional cross-linking polymer relative to the amount of the azetidinium-reactive polymer is from about 0.5 to about 25 dry weight percent on a solids basis.

In another aspect, the invention resides in a method of increasing the strength of a fibrous web comprising topically applying an aqueous binder composition to one or both outer surfaces of the web, wherein the binder composition comprises an unreacted mixture of an azetidinium-reactive polymer and an azetidinium-functional cross-linking polymer, wherein the amount of the azetidinium-functional cross-linking polymer relative to the amount of the azetidinium-reactive polymer is from about 0.5 to about 25 dry weight percent on a solids basis. The treated web can thereafter be optionally creped.

In another aspect, the invention resides in a fibrous web or sheet having first and second outer surfaces, wherein at least one outer surface comprises a topically-applied network of a cured binder composition resulting from the cross-linking reaction of an azetidinium-reactive polymer and an azetidinium-functional cross-linking polymer. As used herein, the term "network" is used to describe any binder pattern that serves to bond the sheet together. The pattern can be regular or irregular and can be continuous or discontinuous.

Products incorporating the fibrous webs of this invention can be single-ply or multi-ply (two, three, or more plies). The binder composition can be applied to one or more surfaces of the ply or plies within the product. For example, a single-ply product can have one or both surfaces treated with the binder composition. A two-ply product can have one or both outer surfaces treated with the binder composition and/or one or both inner surfaces treated with the binder composition. In the case of a two-ply product, it can be advantageous to have one or both binder-treated surfaces plied inwardly in order to expose the untreated surface(s) of the plies on the outside of the product for purposes of hand-feel or absorbency. When the binder is applied to the inner surfaces of a multi-ply product, the binder also provides a means of bonding the plies together. In such cases, mechanical bonding may not be required. In the case of a three-ply product, the same options are available. In addition, for example, it may be desirable to provide a center ply which is not treated with binder while the two outer plies are treated with binder as described above.

As used herein, a "polymer" is a macromolecule consisting of at least five monomer units. More particularly, the degree of polymerization, which is the number of monomer units in an average polymer unit for a given sample, can be about 10 or greater, more specifically about 30 or greater, more specifically about 50 or greater and still more specifically from about 10 to about 10,000.

Azetidinium-reactive polymers suitable for use in accordance with this invention are those polymers containing functional pendant groups that will react with azetidinium-functional molecules. Such reactive functional groups include

carboxyl groups, amines and others. Particularly suitable azetidinium-reactive polymers include carboxyl-functional latex emulsion polymers. More particularly, carboxyl-functional latex emulsion polymers useful in accordance with this invention can comprise aqueous emulsion addition copolymerized unsaturated monomers, such as ethylenic monomers, polymerized in the presence of surfactants and initiators to produce emulsion-polymerized polymer particles. Unsaturated monomers contain carbon-to-carbon double bond unsaturation and generally include vinyl monomers, styrenic monomers, acrylic monomers, allylic monomers, acrylamide monomers, as well as carboxyl functional monomers. Vinyl monomers include vinyl esters such as vinyl acetate, vinyl propionate and similar vinyl lower alkyl esters, vinyl halides, vinyl aromatic hydrocarbons such as styrene and substituted styrenes, vinyl aliphatic monomers such as alpha olefins and conjugated dienes, and vinyl alkyl ethers such as methyl vinyl ether and similar vinyl lower alkyl ethers. Acrylic monomers include lower alkyl esters of acrylic or methacrylic acid having an alkyl ester chain from one to twelve carbon atoms as well as aromatic derivatives of acrylic and methacrylic acid. Useful acrylic monomers include, for instance, methyl, ethyl, butyl, and propyl acrylates and methacrylates, 2-ethyl hexyl acrylate and methacrylate, cyclohexyl, decyl, and isodecyl acrylates and methacrylates, and similar various acrylates and methacrylates.

In accordance with this invention, the carboxyl-functional latex emulsion polymer can contain copolymerized carboxyl-functional monomers such as acrylic and methacrylic acids, fumaric or maleic or similar unsaturated dicarboxylic acids, where the preferred carboxyl monomers are acrylic and methacrylic acid. The carboxyl-functional latex polymers comprise by weight from about 1% to about 50% copolymerized carboxyl monomers with the balance being other copolymerized ethylenic monomers. Preferred carboxyl-functional polymers include carboxylated vinyl acetate-ethylene terpolymer emulsions such as Airflex® 426 Emulsion, commercially available from Air Products Polymers, LP.

Suitable azetidinium-functional cross-linking polymers include polyamide-epichlorohydrin (PAE) resins, polyamide-polyamine-epichlorohydrin (PPE) resins, polydiallylamine-epichlorohydrin resins and other such resins generally produced via the reaction of an amine-functional polymer with an epihalohydrin. Many of these resins are described in the text "Wet Strength Resins and Their Applications", chapter 2, pages 14-44, TAPPI Press (1994), herein incorporated by reference.

The relative amounts of the azetidinium-reactive polymer and the azetidinium-functional cross-linking polymer will depend on the number of functional groups (degree of functional group substitution on molecule) present on each component. In general, it has been found that properties desirable for a disposable paper towel, for example, are achieved when the level of azetidinium-reactive polymer exceeds that of the azetidinium-functional cross-linking polymer on a dry solids basis. More specifically, on a dry solids basis, the amount of azetidinium-functional cross-linking polymer relative to the amount of azetidinium-reactive polymer can be from about 0.5 to about 25 weight percent, more specifically from about 1 to about 20 weight percent, still more specifically from about 2 to about 10 weight percent and still more specifically from about 5 to about 10 weight percent. Other applications may require higher levels of azetidinium-functional cross-linking polymer to achieve desired end use properties.

The surface area coverage of the binder composition on the fibrous web can be about 5 percent or greater, more specifically about 30 percent or greater, still more specifically from

about 5 to about 90 percent, and still more specifically from about 20 to about 75 percent. The binder composition can be applied to one or both surfaces of the fibrous web by any suitable method such as printing, spraying, coating, foaming and the like.

Curing temperatures for the binder composition can be about 260° C. or less, more specifically about 120° C. or less, more specifically about 100° C. or less, more specifically about 40° C. or less, more specifically from about 10 to about 10 260° C. and still more specifically from about 20 to about 120° C. It will be appreciated that although the binder compositions of this invention can be cured at relatively low temperatures, the rate of curing can be accelerated at higher temperatures associated with curing conventional binders. 15 However, such higher cure temperatures are not necessary with the binder compositions of this invention.

The "wet/dry ratio" for paper towels in accordance with this invention, which is the ratio of the CD wet tensile strength divided by the CD dry tensile strength for a given towel 20 sample, can be about 0.40 or greater, more specifically from about 0.40 to about 0.70, and still more specifically from about 0.45 to about 0.65.

Although the binder compositions of this invention have very desirable anti-blocking characteristics, the binder compositions of this invention can optionally contain anti-blocking additives designed to modify the surface chemistry or characteristics of the binder film on the basesheet. Suitable anti-blocking additives include: 1) chemically reactive additives, such as multifunctional aldehydes, including glyoxal, 25 glutaraldehyde and glyoxalated polyacrylamides designed to increase the level of crosslinking of the latex polymer immediately after drying the web; 2) non-reactive additives, such as silicones, waxes, oils, designed to modify the surface chemistry of at least one outer surface of the web to reduce blocking; and 3) soluble or insoluble crystals, such as sugars, talc, 30 clay and the like, designed to reside on the surface of the binder film and thus reduce its propensity to cause blocking to an adjacent web surface. The amount of the anti-blocking additive in the binder composition, relative to the amount of azetidinium-reactive polymer on a weight percent solids basis, can be from about 1 to about 25 percent, more specifically from about 5 to about 20 percent and more specifically from about 10 to about 15 percent.

The effectiveness of an anti-blocking additive can be measured in accordance with the Blocking Test (hereinafter defined). Blocking test values for fibrous sheets, particularly paper towels, in accordance with this invention can be about 45 23 grams (force) or less, more specifically about 20 grams (force) or less, more specifically from about 1 to about 23 50 grams (force) and still more specifically from about 1 to about 15 grams (force).

#### Test Methods

55 As used herein, the "machine direction (MD) tensile strength" represents the peak load per sample width when a sample is pulled to rupture in the machine direction. In comparison, the cross-machine direction (CD) tensile strength represents the peak load per sample width when a sample is pulled to rupture in the cross-machine direction. Unless specified otherwise, tensile strengths are dry tensile strengths.

Samples for tensile strength testing are prepared by cutting a 3 inches (76.2 mm) wide×5 inches (127 mm) long strip in either the machine direction (MD) or cross-machine direction (CD) orientation using a JDC Precision Sample Cutter (Thwing-Albert Instrument Company, Philadelphia, Pa., Model No. JDC 3-10, Serial No. 37333). The instrument used

for measuring tensile strengths is an MTS Systems Sintech 11S, Serial No. 6233. The data acquisition software is MTS TestWorks® for Windows Ver. 3.10 (MTS Systems Corp., Research Triangle Park, N.C.). The load cell is selected from either a 50 Newton or 100 Newton maximum, depending on the strength of the sample being tested, such that the majority of peak load values fall between 10-90% of the load cell's full scale value. The gauge length between jaws is 4+/-0.04 inches (101.6+/-1 mm). The jaws are operated using pneumatic-action and are rubber coated. The minimum grip face width is 3 inches (76.2 mm), and the approximate height of a jaw is 0.5 inches (12.7 mm). The crosshead speed is 10+/-0.4 inches/min (254+/-1 mm/min), and the break sensitivity is set at 65%. The sample is placed in the jaws of the instrument, centered both vertically and horizontally. The test is then started and ends when the specimen breaks. The peak load is recorded as either the "MD tensile strength" or the "CD tensile strength" of the specimen depending on the sample being tested. At least six (6) representative specimens are tested for each product and the arithmetic average of all individual specimen tests is either the MD or CD tensile strength for the product.

Wet tensile strength measurements are measured in the same manner, but are only typically measured in the cross-machine direction of the sample. Prior to testing, the center portion of the CD sample strip is saturated with room temperature tap water immediately prior to loading the specimen into the tensile test equipment. CD wet tensile measurements can be made both immediately after the product is made and also after some time of natural aging of the product. For mimicking natural aging, experimental product samples are stored at ambient conditions of approximately 23° C. and 50% relative humidity for up to 15 days or more prior to testing so that the sample strength no longer increases with time. Following this natural aging step, the samples are individually wetted and tested. Alternatively, samples may be tested immediately after production with no additional aging time. For these samples, the tensile strips are artificially aged for 5 or 10 minutes in an oven at 105° C. prior to testing. Following this artificial aging step, the samples are individually wetted and tested. For measuring samples that have been made more than two weeks prior to testing, which are inherently naturally aged, such conditioning is not necessary.

Sample wetting is performed by first laying a single test strip onto a piece of blotter paper (Fiber Mark, Reliance Basis 120). A pad is then used to wet the sample strip prior to testing. The pad is a Scotch-Brite® brand (3M) general purpose commercial scrubbing pad. To prepare the pad for testing, a full-size pad is cut approximately 2.5 inches (63.5 mm) long by 4 inches (101.6 mm) wide. A piece of masking tape is wrapped around one of the 4 inch (101.6 mm) long edges. The taped side then becomes the "top" edge of the wetting pad. To wet a tensile strip, the tester holds the top edge of the pad and dips the bottom edge in approximately 0.25 inch (6.35 mm) of tap water located in a wetting pan. After the end of the pad has been saturated with water, the pad is then taken from the wetting pan and the excess water is removed from the pad by lightly tapping the wet edge three times on a wire mesh screen. The wet edge of the pad is then gently placed across the sample, parallel to the width of the sample, in the approximate center of the sample strip. The pad is held in place for approximately one second and then removed and placed back into the wetting pan. The wet sample is then immediately inserted into the tensile grips so the wetted area is approximately centered between the upper and lower grips. The test strip should be centered both horizontally and vertically between the grips. (It should be noted that if any of the wetted

portion comes into contact with the grip faces, the specimen must be discarded and the jaws dried off before resuming testing.) The tensile test is then performed and the peak load recorded as the CD wet tensile strength of this specimen. As with the dry tensile tests, the characterization of a product is determined by the average of six representative sample measurements.

In addition to tensile strength, stretch is also reported by the MTS TestWorks® for Windows Ver. 3.10 program for each sample measured. Stretch is reported as a percentage and is defined as the ratio of the slack-corrected elongation of a specimen at the point it generates its peak load divided by the slack-corrected gage length.

As used herein, the Blocking Test value is determined by ASTM D 5170-98-Standard Test Method for Peel Strength ("T" Method) of Hook and Loop Touch Fasteners, but with the following exceptions in order to adapt the method from hook and loop testing to tissue testing (modified ASTM section numbers are shown in parenthesis):

- 20 (a) Replace all references to "hook and loop touch fasteners" with "blocked tissue samples".
- (b) (Section 3.3) Only one calculation method is used, namely the "integrator average" or average force over the measured distance.
- 25 (c) (Section 4.1) No roller device is used.
- (d) (Section 6. Specimen Preparation) Replace all contents with the following:

The level of blocking that will occur naturally over prolonged aging under pressure in a wound roll can be simulated by conditioning the samples in an oven under pressure. To artificially block samples, the 2 sheet specimens to be blocked together are cut to 76.2+/-1 mm (3+/-0.04 inches) in the cross direction by 177.8+/-25.4 mm (7+/-1 inch) in the machine direction. The specimens are then placed on a flat surface in an oven operating at 66° C. On top of the specimens is placed a lightweight polycarbonate plate. On top of the polycarbonate plate, centered on the sample strips, is placed an iron block weighing approximately 11,800 g and having a bottom face area of 10.2 cm x 10.2 cm. The samples are stored in the oven under the applied weight for 1 hour. When the samples are removed from the oven, they are allowed to equilibrate under no additional weight for at least 4 hours in standard TAPPI conditions (25° C. and 50% relative humidity) prior to conducting the blocking test.

- 45 (e) (Section 8. Procedure) Replace all contents with the following:

"Separate the top and bottom sheet of the specimen along the CD (3 inch) edge. Peel back approximately 51 mm (2 inches) of the top and bottom sheets in the machine direction.

50 Position the clamps of the tensile tester so they are 25.4+/-1 mm (1+/-0.04 inches) apart. Place the free ends of the specimen to be tested in the clamps of the tensile tester, with the specimen tail facing away from the frame. The point of specimen separation should be approximately centered between the clamps and aligned approximately parallel to the clamps. For the integrator calculation, set up the software to begin averaging after 25.4 mm (1 inch) of separation and end averaging after 88.9 mm (3.5 inches) of separation. The software should be set up to separate the sample over a total of 101.6 mm (4 inches)."

- 60 (f) (Section 9. Calculation) Omit all but 9.2.
- (g) (Section 10. Report) Replace all contents with the following:

"Report the integrator average for each specimen."

- 65 (h) (Section 11.1) Replace all contents with the following:
- "At least 5 specimens should be tested for a reliable sample average."

As used herein, "bulk" is calculated as the quotient of the caliper (hereinafter defined) of a product, expressed in microns, divided by the basis weight, expressed in grams per square meter. The resulting bulk of the product is expressed in cubic centimeters per gram. Caliper is measured as the total thickness of a stack of ten representative sheets of product and dividing the total thickness of the stack by ten, where each sheet within the stack is placed with the same side up. Caliper is measured in accordance with TAPPI test methods T402 "Standard Conditioning and Testing Atmosphere For Paper, Board, Pulp Handsheets and Related Products" and T411 om-89 "Thickness (caliper) of Paper, Paperboard, and Combined Board" with Note 3 for stacked sheets. The micrometer used for carrying out T411 om-89 is an Emveco 200-A Tissue Caliper Tester available from Emveco, Inc., Newberg, Oreg. The micrometer has a load of 2.00 kilo-Pascals (132 grams per square inch), a pressure foot area of 2500 square millimeters, a pressure foot diameter of 56.42 millimeters, a dwell time of 3 seconds and a lowering rate of 0.8 millimeters per second. After the caliper is measured, the top sheet of the stack of 10 is removed and the remaining sheets are used to determine the basis weight.

The products (single-ply or multi-ply) or sheets of this invention can have a bulk of about 11 cubic centimeters or greater per gram, more specifically about 12 cubic centimeters or greater per gram, more specifically about 13 cubic centimeters or greater per gram, more specifically from about 11 to about 20 cubic centimeters per gram, and still more specifically from about 12 to about 20 cubic centimeters per gram. Particular products of this invention include paper towels, bath tissue, facial tissue, table napkins, wipes and the like.

#### BRIEF DESCRIPTION OF THE DRAWING

FIG. 1 is a schematic flow diagram of a process for topically applying a binder or binders to a paper web in accordance with this invention.

#### DETAILED DESCRIPTION OF THE DRAWINGS

Referring to FIG. 1, shown is a method of applying a topical binder material to a previously-formed basesheet or web. The binder material can be applied to one or both sides of the web. For wet laid basesheets, at least one side of the web is thereafter creped. In general, for most applications, the basesheet or web will only be creped on one side after the binder materials are applied. It should be understood, however, that in some situations it may be desirable to crepe both sides of the web. Alternatively, nonwoven manufacturing processes which may not contain a creping step, such as air-laid papermaking processes, for example, may also utilize the low odor binder of the present invention for imparting structural integrity to the web. In such cases, post-treatment with topical binder material is optional.

Prior to applying the binder material to the web, the azetidinium-reactive polymer and the azetidinium-functional polymer can be mixed together along with any other binder formulation ingredients. Consequently, the binder material may be prepared in different ways, but a convenient method of preparation is to simply blend the azetidinium-functional polymer with the azetidinium-reactive polymer, water, defoamer (optional), pH control chemistry (optional) and anti-blocking additive (optional) and the resulting blended binder formulation is applied to the fibrous web, such as by printing, spraying, coating, foaming, size pressing or other means. Depending upon the stability of the resulting blended binder formulation, the elapsed time between blending of the

binder composition and its application to the web can be less than a week, more specifically 48 hours or less, more specifically 24 hours or less, and still more specifically about 4 hours or less.

5 Returning to FIG. 1, a fibrous web 10 made according to any suitable wet-laying or air-laying process is passed through a first binder material application station 12. Station 12 includes a nip formed by a smooth rubber press roll 14 and a patterned rotogravure roll 16. Rotogravure roll 16 is in communication with a reservoir 18 containing a first binder material 20. The rotogravure roll applies the binder material to one side of web in a pre-selected pattern.

10 Web 10 is then contacted with a heated roll 22 after passing a roll 24. The heated roll 22 serves to at least partially dry the web. The heated roll can be heated to a temperature, for instance, up to about 121° C. and particularly from about 82° C. to about 104° C. In general, the web can be heated to a temperature sufficient to dry the web and evaporate any water. During the time the web is heated, some curing of the binder 15 on the sheet may occur.

20 It should be understood, that the besides the heated roll 22, any suitable heating device can be used to dry the web. For example, in an alternative embodiment, the web can be placed in communication with a through-air dryer or an infra-red 25 heater in order to dry the web. Other heating devices can include, for instance, any suitable convective oven, microwave oven or other suitable electromagnetic wave energy source.

20 From the heated roll 22, the web 10 can be advanced by pull 30 rolls 26 to a second binder material application station generally 28. Station 28 includes a transfer roll 30 in contact with a rotogravure roll 32, which is in communication with a reservoir 34 containing a second binder material 36. Similar to station 12, second binder material 36 is applied to the 35 opposite side of web 10 in a pre-selected pattern. Once the second binder material is applied, web 10 is adhered to a creping roll or drum 38 by a press roll 40. The web is carried on the surface of the creping roll for a distance and then removed therefrom by the action of a creping blade 42. The 40 creping blade performs a controlled pattern creping operation on the second side of the paper web.

45 In accordance with the present invention, the second binder material 36 is selected such that the web 10 can be adhered to and creped from the creping drum 38. For example, in accordance with the present invention, the creping drum can be maintained at a temperature of between 66° C. and 121° C. Operation outside of this range is also possible. In one embodiment, for example, the creping drum 108 can be at 104° C. Alternatively, the creping drum need not be heated or 50 only heated to a relatively low temperature.

55 Once creped, the paper web 10 is pulled through a drying station 44. Drying station 44 can include any form of a heating unit, such as an oven energized by infrared heat, microwave energy, hot air or the like. Alternatively, the drying station 60 may comprise other drying methods such as photo-curing, UV-curing, corona discharge treatment, electron beam curing, curing with reactive gas, curing with heated air such as through-air heating or impingement jet heating, infrared heating, contact heating, inductive heating, microwave or RF heating, and the like. The dryer may also include a fan to blow air onto the moving web. Drying station 44 may be necessary in some applications to dry the web and/or cure the first and second binder materials. Depending upon the binder materials selected, however, in other applications the drying station 65 may not be needed.

The amount that the paper web is heated within the drying station 44 can depend upon the particular binder materials

used, the amount of binder materials applied to the web, and the type of web used. In some applications, for instance, the paper web can be heated using a gas stream such as air at a temperature of about 265° C. in order to cure the binder materials. When using low cure temperature binder materials, on the other hand, the gas can be at a temperature lower than about 130° C. and particularly lower than about 120° C. In an alternative embodiment, the drying station 44 is not used to cure the binder material applied to the web. Instead, the drying station is used to dry the web and to drive off any water present in the web. In this embodiment, the web can be heated to temperatures sufficient to evaporate water, such as to a temperature of from about 90 to about 120° C. In other embodiments, room temperature air (20-40° C.) may be sufficient to dry the web. In still other embodiments, the drying station may be bypassed or removed from the process altogether.

Once passed through drying station, web 10 can be wound into a roll of material 46 for subsequent conversion into the final product. In other embodiments, the web may proceed directly into further converting operations to result in the final product without being wound into an intermediate roll.

## EXAMPLES

### Example 1

#### Epoxy-Functional Reactant Control

In general, a single-ply uncreped through-air-dried (UC-TAD) sheet was produced generally as described in U.S. Pat. No. 5,593,545 issued Jan. 14, 1997 to Rugowski et al., herein incorporated by reference. After manufacture on the tissue machine, the UCTAD basesheet was printed on each side with a latex-based binder. The binder-treated sheet was adhered to the surface of a Yankee dryer to re-dry the sheet and thereafter the sheet was creped and wound onto a roll without any additional thermal curing. The resulting sheet was tested for physical properties after natural aging at room temperature (about 23° C.) and humidity (about 50% relative humidity).

More specifically, the basesheet was made from a stratified fiber furnish containing a center layer of fibers positioned between two outer layers of fibers. Both outer layers of the UCTAD basesheet contained 100% northern softwood kraft pulp and about 3.5 kilograms (kg)/metric ton (Mton) of dry fiber of a debonding agent, ProSoft® TQ1003 (Hercules, Inc.). Combined, the outer layers comprised 50% of the total fiber weight of the sheet (25% in each layer). The center layer, which comprised 50% of the total fiber weight of the sheet, was also comprised of northern softwood kraft pulp. The fibers in this layer were also treated with 3.5 kg/Mton of ProSoft® TQ1003 debonder.

The machine-chest furnish containing the chemical additives was diluted to approximately 0.2 percent consistency and delivered to a layered headbox. The forming fabric speed was approximately 445 meters per minute. The resulting web was then rush-transferred to a transfer fabric (Voith Fabrics, 807) traveling 15% slower than the forming fabric using a vacuum box to assist the transfer. At a second vacuum-assisted transfer, the web was transferred and wet-molded onto the through-drying fabric (Voith Fabrics, t1203-8). The web was dried with a through-air-dryer resulting in a basesheet with an air-dry basis weight of approximately 45 grams per square meter (gsm).

The resulting sheet was fed to a gravure printing line, similar to that shown in FIG. 1, traveling at about 200 feet per minute (61 meters per minute) where a latex binder was

printed onto the surface of the sheet. The first side of the sheet was printed with a bonding formulation using direct rotogravure printing. Then the printed web passed over a heated roll with a surface temperature of approximately 104° C. to evaporate water. Next, the second side of the sheet was printed with the bonding formulation using a second direct rotogravure printer. The sheet was then pressed against and doctored off a rotating drum, which had a surface temperature of approximately 104° C. Finally the sheet was cooled by passing room temperature air through the sheet prior to winding into a roll. The temperature of the wound roll was measured to be approximately 24° C.

The bonding formulation for this example was prepared as two separate mixtures, called the "latex" and "reactant". The "latex" material contained the epoxy-reactive polymer and the "reactant" was the epoxy-functional polymer. Each mixture was made up independently and then combined together prior to use. After the latex and reactant mixtures were combined, the appropriate amount of "thickener" (Natrosol solution) was added to adjust viscosity. The "latex" and "reactant" mixtures contained the following ingredients, listed in their order of addition.

| Latex                                |         |
|--------------------------------------|---------|
| 1. Airflex ® 426 (62.7% solids)      | 8,555 g |
| 2. Defoamer (Nalco 7565)             | 50 g    |
| 3. Water                             | 1,530 g |
| 4. LiCl solution tracer (10% solids) | 50 g    |
| Reactant                             |         |
| 1. Kymene ® 2064 (20% solids)        | 1,356 g |
| 2. Water                             | 2,000 g |
| 3. NaOH (10% solution)               | 700 g   |

When the NaOH had been added, the pH of the reactant mixture was approximately 12. After all reactant ingredients were added, the mixture was allowed to mix for at least 15 minutes prior to adding to the latex mixture.

| Thickener                               |       |
|-----------------------------------------|-------|
| 1. Natrosol 250MR, Hercules (2% solids) | 600 g |

After all ingredients had been added, the print fluid was allowed to mix for approximately 5-30 minutes prior to use in the gravure printing operation. For this bonding formulation, the weight percent ratio of epoxy-functional polymer based on carboxylic acid-functional polymer (epoxy-reactive polymer) was about 5%.

Lithium Chloride (LiCl) salt was added to the bonding formulation as a tracer to enable latex addition level to be analyzed using atomic absorption spectroscopy. An amount of LiCl no less than 250 parts per million (ppm) was added in the bonding formulation to ensure accurate detection measurement. The LiCl granules were dissolved in water and then added to the bonding formulation under agitation. After applying the bonding formulation to a basesheet, a sample of the bonding formulation and also a sample of the bonded sheet were collected for analysis.

The bonding formulation and bonded sheet were analyzed using atomic absorption spectroscopy to determine the percentage of latex add-on. First a calibration curve of absorbance vs. lithium concentration in ppm was created with standard LiCl solutions in water. The bonding formulations

## 11

and bonded sheet were analyzed with atomic absorption spectroscopy after undergoing a series of combustion and water extraction steps to capture all lithium ions present in the respective samples. The weights of LiCl in the bonding formulation and bonded sheet samples were obtained by comparing their atomic absorbance values to the LiCl calibration curve. The concentration of LiCl in the bonding formulation was calculated, and then the weight of LiCl in each bonded sheet sample was converted into the amount of bonding formulation (W<sub>t</sub>(BF)) applied to the sheet based on the LiCl content in the bonding formulation. Since the total solids content of the bonding formulation, S<sub>T</sub>, and latex solids content, S<sub>L</sub>, in the total solids are known, the percent of latex solids add-on (Latex %) can be calculated using the following equation:

$$\text{Latex \%} = \frac{W_t(\text{BF}) \times S_T \times S_L}{W_t(\text{Sample})} \times 100$$

where W<sub>t</sub>(BF) is the weight of bonding formulation applied to the sheet in milligrams (mg), W<sub>t</sub>(Sample) is the weight of bonded sheet in mg, S<sub>T</sub> is the weight percent content of total solids in the bonding formulation, and S<sub>L</sub> is the weight percent of latex solids in the total solids.

The viscosity of the print fluid was 120 cps, when measured at room temperature using a viscometer (Brookfield® Synchro-lectric viscometer Model RVT, Brookfield Engineering Laboratories Inc. Stoughton, Mass.) with a #1 spindle operating at 20 rpm. The oven-dry solids of the print fluid was 38 weight percent. The print fluid pH was 3.7.

Thereafter the print/print/creped sheet was removed from the roll and tested for basis weight, tensile strength and sheet blocking. Wet tensile testing was conducted after first artificially aging the sheet for 10 minutes in an oven operating at 105° C. Approximately 6% by weight Airflex® 426 was applied to the sheet.

## Example 2

## Invention

A single-ply bonded sheet was produced as described in Example 1, but using a different binder recipe. For this example, an azetidinium-functional reactant, Kymene® 557LX (Hercules Inc., Wilmington, Del.) was used. The ingredients of the "latex", "reactant" and "thickener" are listed below.

| <u>Latex</u>                            |         |
|-----------------------------------------|---------|
| 1. Airflex ® 426 (62.7% solids)         | 8,555 g |
| 2. Defoamer (Nalco 7565)                | 54 g    |
| 3. Water                                | 1,530 g |
| 4. LiCl solution tracer (10% solids)    | 65 g    |
| Reactant                                |         |
| 1. Kymene ® 557LX (12.5% solids)        | 1,356 g |
| 2. Water                                | 1,875 g |
| Thickener                               |         |
| 1. Natrosol 250MR, Hercules (2% solids) | 700 g   |

The reactant ingredients (Kymene and water) were added directly to the Latex mixture under agitation. After all ingredients had been added, the print fluid was allowed to mix for approximately 5-30 minutes prior to use in the gravure printing operation. For this bonding formulation, the weight percent ratio of azetidinium-functional polymer based on carboxylic acid-functional polymer was 3.2%.

5 The viscosity of the print fluid was 125 cps, when measured at room temperature using a viscometer (Brookfield® Synchro-lectric viscometer Model RVT, Brookfield Engineering Laboratories Inc. Stoughton, Mass.) with a #1 spindle operating at 20 rpm. The oven-dry solids of the print fluid was 38.2 weight percent. The print fluid pH was 3.7.

10 Thereafter the print/print/creped sheet was removed from the roll and tested for basis weight, tensile strength and sheet blocking. Wet tensile testing was conducted after first artificially aging the sheet for 10 minutes in an oven operating at 15 105° C. Approximately 6% by weight Airflex® 426 was applied to the sheet.

## Example 3

## Invention

A single-ply bonded sheet was produced as described in Example 2, but using a binder recipe which was designed to reduce blocking in the finished roll. The ingredients of the "latex", "reactant", "anti-blocking additive" and "thickener" are listed below.

| <u>Latex</u>                         |         |
|--------------------------------------|---------|
| 1. Airflex ® 426 (62.7% solids)      | 6,920 g |
| 2. Defoamer (Nalco 7565)             | 40 g    |
| 3. Water                             | 5,485 g |
| 4. LiCl solution tracer (10% solids) | 40 g    |
| Reactant                             |         |
| 1. Kymene ® 557LX (12.5% solids)     | 2,180 g |

30 The reactant was added directly to the latex mixture under agitation. After all ingredients had been added, the print fluid was allowed to mix for approximately 5-30 minutes.

40 The anti-blocking additive was added next, followed by the thickener to achieve desired viscosity.

| <u>Anti-Blocking Additive</u>           |         |
|-----------------------------------------|---------|
| 1. Glyoxal (40%)                        | 548 g   |
| Thickener                               |         |
| 1. Natrosol 250MR, Hercules (2% solids) | 1,010 g |

45 After all ingredients had been added, the print fluid was allowed to mix for approximately 5-30 minutes prior to use in the gravure printing operation. For this bonding formulation, the weight percent ratio of azetidinium-functional polymer based on carboxylic acid-functional polymer was 6.25% and the weight percent ratio of glyoxal based on carboxylic acid-functional polymer was about 5%. The viscosity of the print fluid was 82.5 cps, when measured at room temperature using a viscometer (Brookfield® Synchro-lectric viscometer Model RVT, Brookfield Engineering Laboratories Inc. Stoughton, Mass.) with a #1 spindle operating at 20 rpm. The print fluid pH was 3.5.

50 The resulting single-ply bonded sheet was tested for tensile strength and sheet blocking after 14 days of aging at room temperature conditions.

**13**  
Example 4

## Invention

A single-ply bonded sheet was produced as described in Example 2, but using a binder recipe which was designed to reduce blocking in the finished roll. The anti-blocking additives used in this example included glyoxal and a glyoxalated polyacrylamide (Parez® 631NC, Bayer Chemicals Corp.) The ingredients of the “latex”, “reactant”, “anti-blocking additives” and “thickener” are listed below.

| <u>Latex</u>                         |         |
|--------------------------------------|---------|
| 1. Airflex ® 426 (62.7% solids)      | 6,920 g |
| 2. Defoamer (Nalco 7565)             | 40 g    |
| 3. Water                             | 3,670 g |
| 4. LiCl solution tracer (10% solids) | 40 g    |
| <u>Reactant</u>                      |         |
| 1. Kymene ® 557LX (12.5% solids)     | 2,175 g |

The reactant was added directly to the latex mixture under agitation. After all ingredients had been added, the print fluid was allowed to mix for approximately 5-30 minutes.

The anti-blocking additives were added next, followed by the thickener to achieve desired viscosity.

| <u>Anti-Blocking Additives</u>          |         |
|-----------------------------------------|---------|
| 1. Glyoxal (40%)                        | 543 g   |
| 2. Parez 631NC (6.0%)                   | 1,816 g |
| <u>Thickener</u>                        |         |
| 1. Natrosol 250MR, Hercules (2% solids) | 220 g   |

After all ingredients had been added, the print fluid was allowed to mix for approximately 5-30 minutes prior to use in the gravure printing operation. For this bonding formulation, the weight percent ratio of azetidinium-functional polymer based on carboxylic acid-functional polymer was 10% and the weight percent ratio of glyoxal and Parez 631NC based on carboxylic acid-functional polymer were 10% and 5%, respectively. The viscosity of the print fluid was 120 cps, when measured at room temperature using a viscometer (Brookfield® Synchro-lectric viscometer Model RVT, Brookfield Engineering Laboratories Inc. Stoughton, Mass.) with a #1 spindle operating at 20 rpm. The print fluid pH was 3.5. The latex binder addition was approximately 6% by weight Airflex® 426 based on the finished sheet.

The resulting single-ply bonded sheet was tested for tensile strength and sheet blocking after 14 days of aging at room temperature conditions.

## Example 5

## Invention

A single-ply bonded sheet was produced as described in Example 2, but using a binder recipe which was designed to reduce blocking in the finished roll. The anti-blocking additives used in this example included glyoxal and a glyoxalated polyacrylamide (Parez® 631NC, Bayer Chemicals Corp.) The ingredients of the “latex”, “reactant”, “anti-blocking additives” and “thickener” are listed below.

| <u>Latex</u>                         |         |
|--------------------------------------|---------|
| 1. Airflex ® 426 (62.7% solids)      | 6,920 g |
| 2. Defoamer (Nalco 7565)             | 40 g    |
| 3. Water                             | 2,000 g |
| 4. LiCl solution tracer (10% solids) | 40 g    |
| <u>Reactant</u>                      |         |
| 1. Kymene ® 557LX (12.5% solids)     | 3,488 g |

The reactant was added directly to the latex mixture under agitation. After all ingredients had been added, the print fluid was allowed to mix for approximately 5-30 minutes.

The anti-blocking additives were added next. No thickener was added to this code.

| <u>Anti-Blocking Additives</u> |         |
|--------------------------------|---------|
| 1. Glyoxal (40%)               | 1,090 g |
| 2. Parez 631NC (6.0%)          | 3,633 g |

After all ingredients had been added, the print fluid was allowed to mix for approximately 5-30 minutes prior to use in the gravure printing operation. For this bonding formulation, the weight percent ratio of azetidinium-functional polymer based on carboxylic acid-functional polymer was 10% and the weight percent ratio of glyoxal and Parez 631NC based on carboxylic acid-functional polymer were 10% and 5%, respectively. The viscosity of the print fluid was 120 cps, when measured at room temperature using a viscometer (Brookfield® Synchro-lectric viscometer Model RVT, Brookfield Engineering Laboratories Inc. Stoughton, Mass.) with a #1 spindle operating at 20 rpm. The print fluid pH was 3.5. The latex binder addition was approximately 6% by weight Airflex® 426 based on the finished sheet.

The resulting single-ply bonded sheet was tested for tensile strength and sheet blocking after 14 days of aging at room temperature conditions.

## Example 6

## Invention

A single-ply bonded sheet was produced as described in Example 2, but using a binder recipe which was designed to reduce blocking in the finished roll. The anti-blocking additives used in this example included glyoxal and a glyoxalated polyacrylamide (Parez® 631NC, Bayer Chemicals Corp.) The ingredients of the “latex”, “reactant”, “anti-blocking additives” and “thickener” are listed below.

| <u>Latex</u>                         |         |
|--------------------------------------|---------|
| 1. Airflex ® 426 (62.7% solids)      | 6,920 g |
| 2. Defoamer (Nalco 7565)             | 52 g    |
| 3. Water                             | 3,153 g |
| 4. LiCl solution tracer (10% solids) | 42 g    |
| <u>Reactant</u>                      |         |
| 1. Kymene ® 557LX (12.5% solids)     | 2,180 g |

The reactant was added directly to the latex mixture under agitation. After all ingredients had been added, the print fluid was allowed to mix for approximately 5-30 minutes.

## 15

The anti-blocking additives were added next. No thickener was added to this code.

| Anti-Blocking Additives |         |
|-------------------------|---------|
| 1. Glyoxal (40%)        | 545 g   |
| 2. Parez 631NC (6.0%)   | 3,634 g |

After all ingredients had been added, the print fluid was allowed to mix for approximately 5-30 minutes prior to use in the gravure printing operation. For this bonding formulation, the weight percent ratio of azetidinium-functional polymer based on carboxylic acid-functional polymer was 6.25% and the weight percent ratio of glyoxal and Parez 631NC based on carboxylic acid-functional polymer were 5% and 5%, respectively. The viscosity of the print fluid was 90 cps, when measured at room temperature using a viscometer (Brookfield® Synchro-lectric viscometer Model RVT, Brookfield Engineering Laboratories Inc. Stoughton, Mass.) with a #1 spindle operating at 20 rpm. The print fluid pH was 3.6. The latex binder addition was approximately 6% by weight Airflex® 426 applied to the sheet.

The resulting single-ply bonded sheet was tested for tensile strength and sheet blocking after 14 days of aging at room temperature conditions.

## Example 7

## Invention with One Print Step

A single-ply UCTAD sheet was produced generally as described in Example 1. After manufacture on the tissue machine, the UCTAD basesheet was printed on one side with a latex-based binder. The binder-treated sheet was adhered to the surface of a Yankee dryer to re-dry the sheet and thereafter the sheet was creped and wound onto a roll without any additional thermal curing. The resulting sheet was tested for physical properties after natural aging at room temperature (about 23° C.) and humidity (about 50% relative humidity).

More specifically, the basesheet was made from a stratified fiber furnish containing a center layer of fibers positioned between two outer layers of fibers. Both outer layers of the UCTAD basesheet contained 100% northern softwood kraft pulp. One outer layer was treated with 8.0 kilograms (kg)/metric ton (Mton) of dry fiber of a debonding agent, ProSoft® TQ1003 (Hercules, Inc.) and the other outer layer was treated with 3.0 kg/Mton of Prosoft® TQ1003. Both outer layers were also treated with 5.0 kg/Mton of a wet strength agent, Kymene 557LX (Hercules, Inc.). Combined, the outer layers comprised 50% of the total fiber weight of the sheet (25% in each layer). The center layer, which comprised 50% of the total fiber weight of the sheet, was also comprised of northern softwood kraft pulp. The fibers in this layer were also treated with 8.0 kg/Mton of ProSoft® TQ1003 debonder.

The machine-chest furnish containing the chemical additives was diluted to approximately 0.2 percent consistency and delivered to a layered headbox. The forming fabric speed was approximately 445 meters per minute. The resulting web was then rush-transferred to a transfer fabric (Voith Fabrics, t1207-6) traveling 25% slower than the forming fabric using a vacuum box to assist the transfer. At a second vacuum-assisted transfer, the web was transferred and wet-molded onto the through-drying fabric (Voith Fabrics, t1207-6). The web was dried with a through-air-dryer resulting in a basesheet with an air-dry basis weight of approximately 48 grams per square meter (gsm).

## 16

The resulting sheet was fed to a gravure printing line, similar to that shown in FIG. 1, traveling at about 1000 feet per minute (305 meters per minute) where a latex binder was printed onto one side of the sheet. The printed side of the sheet was then pressed against and doctored off a rotating drum, which had a surface temperature of approximately 84° C. Finally the sheet was wound onto a roll without any additional thermal curing. The temperature of the wound roll was measured to be approximately 36° C.

The bonding formulation for this example contained a "latex", "reactant", "anti-blocking additive" and "pH control chemistry", as listed below in their order of addition.

| Latex                                |          |
|--------------------------------------|----------|
| 1. Airflex ® 426 (63.36% solids)     | 27,680 g |
| 2. Defoamer (Nalco 7565)             | 173 g    |
| 3. Water                             | 5,600 g  |
| 4. LiCl solution tracer (10% solids) | 178 g    |
| Reactant                             |          |
| 1. Kymene ® 557LX (12.5% solids)     | 8,770 g  |
| Anti-Blocking Additive               |          |
| 1. Parez 631NC (6.0%)                | 7,315 g  |
| pH Control Chemistry                 |          |
| 1. NaOH (10% solution)               | 974 g    |

When the NaOH had been added, the pH of the reactant mixture was approximately 6.

After all ingredients had been added, the print fluid was allowed to mix for approximately 5-30 minutes prior to use in the gravure printing operation. For this bonding formulation, the weight percent ratio of azetidinium-functional polymer based on carboxylic acid-functional polymer (azetidinium-reactive polymer) was about 6.25%.

The viscosity of the print fluid was 140 cps, when measured at room temperature using a viscometer (Brookfield® Synchro-lectric viscometer Model RVT, Brookfield Engineering Laboratories Inc. Stoughton, Mass.) with a #1 spindle operating at 20 rpm. The oven-dry solids of the print fluid was 38.4 weight percent. The print fluid pH was 6.0.

Thereafter the print/creped sheet was removed from the roll and tested for basis weight, tensile strength and sheet blocking. Wet tensile testing was conducted after first artificially aging the sheet for 5 minutes in an oven operating at 105° C. Approximately 6% by weight Airflex® 426 was applied to the sheet.

A summary of the results of the foregoing Examples 1-7 is set forth in Table 1 below:

TABLE 1

| Ex-<br>am-<br>ple   | MD                |                      | CD                |                      | CD Wet                        |                      | Wet/<br>Dry<br>Ratio   | Blocking<br>Test* |
|---------------------|-------------------|----------------------|-------------------|----------------------|-------------------------------|----------------------|------------------------|-------------------|
|                     | Tensile<br>(g/3") | MD<br>Stretch<br>(%) | Tensile<br>(g/3") | CD<br>Stretch<br>(%) | Tensile<br>Strength<br>(g/3") | Wet/<br>Dry<br>Ratio |                        |                   |
| 1<br>(Con-<br>trol) | 1818              | 42                   | 1458              | 18                   | 593                           | 40%                  | 25<br>(est-<br>imated) |                   |
| 2                   | 1585              | 36                   | 1248              | 17                   | 591                           | 47%                  | Not<br>measured        |                   |
| 3                   | 1213              | 40                   | 1116              | 13                   | 541                           | 48%                  | 3.3                    |                   |
| 4                   | 1377              | 40                   | 1142              | 12                   | 526                           | 46%                  | 5.6                    |                   |
| 5                   | 1326              | 39                   | 1239              | 12                   | 565                           | 46%                  | 3.8                    |                   |

TABLE 1-continued

| Ex-<br>am-<br>ple | MD                            |                      | CD                            |                      | CD Wet                        |     | Wet/<br>Dry<br>Ratio | Blocking<br>Test*<br>(g) |
|-------------------|-------------------------------|----------------------|-------------------------------|----------------------|-------------------------------|-----|----------------------|--------------------------|
|                   | Tensile<br>Strength<br>(g/3") | MD<br>Stretch<br>(%) | Tensile<br>Strength<br>(g/3") | CD<br>Stretch<br>(%) | Tensile<br>Strength<br>(g/3") |     |                      |                          |
| 6                 | 1465                          | 42                   | 1455                          | 12                   | 660                           | 45% | 2.8                  |                          |
| 7                 | 1394                          | 32                   | 966                           | 22                   | 629                           | 65% | Not<br>measured      |                          |

\*blocking values were tested after conditioning samples in an oven at 66° C., under weight which produced 1.44 psi pressure, for 1 hour to simulate blocking in a parent roll.

The data in Table 1 demonstrates the ability of the inventive low cure temperature binder to produce paper with a high level of wet tensile strength, a high wet/dry tensile ratio and a low Blocking Test value.

In the interests of brevity and conciseness, any ranges of values set forth in this specification are to be construed as written description support for claims reciting any sub-ranges having endpoints which are whole number values within the specified range in question. By way of a hypothetical illustrative example, a disclosure in this specification of a range of 1-5 shall be considered to support claims to any of the following sub-ranges: 1-4; 1-3; 1-2; 2-5; 2-4; 2-3; 3-5; 3-4; and 4-5.

It will be appreciated that the foregoing examples, given for purposes of illustration, are not to be construed as limiting the scope of this invention, which is defined by the following claims and all equivalents thereto.

We claim:

1. An aqueous binder composition comprising an unreacted mixture of a carboxylated vinyl acetate-ethylene terpolymer emulsion, a polyamide-polyamine-epichlorohydrin resin and an anti-blocking additive, wherein the amount of the polyamide-polyamine-epichlorohydrin resin relative to the amount of the carboxylated vinyl acetate-ethylene terpolymer emulsion is from about 0.5 to about 25 dry weight percent on a solids basis and wherein the amount of the anti-blocking additive is from about 1 to about 25 weight percent, on a solids basis, relative to the amount of the carboxylated vinyl acetate-ethylene terpolymer, wherein the anti-blocking additive is selected from the group consisting of glyoxal, gluteraldehyde and sugars.

2. The composition of claim 1 wherein the amount of the polyamide-polyamine-epichlorohydrin resin relative to the amount of the carboxylated vinyl acetate-ethylene terpolymer emulsion is from about 1 to about 20 dry weight percent.

3. The composition of claim 1 wherein the amount of the polyamide-polyamine-epichlorohydrin resin relative to the amount of the carboxylated vinyl acetate-ethylene terpolymer emulsion is from about 2 to about 10 dry weight percent.

4. The composition of claim 1 wherein the amount of the polyamide-polyamine-epichlorohydrin resin relative to the

amount of the carboxylated vinyl acetate-ethylene terpolymer emulsion is from about 5 to about 10 dry weight percent.

5. The method of claim 1 wherein the amount of the anti-blocking additive is from about 5 to about 20 weight percent.

6. The method of claim 1 wherein the amount of the anti-blocking additive is from about 10 to about 15 weight percent.

7. The method of claim 1 wherein the anti-blocking additive is glyoxal.

8. The method of claim 1 wherein the anti-blocking additive is glutaraldehyde.

9. The method of claim 1 wherein the anti-blocking additive is a soluble or insoluble crystal selected from the group consisting of sugars.

10 15 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9